

Patented June 29, 1926.

1,590,196

# UNITED STATES PATENT OFFICE.

ALBERT L. KLEES, OF NEW YORK, N. Y., ASSIGNOR TO COMBUSTION UTILITIES CORPORATION, OF NEW YORK, N. Y., A CORPORATION OF MAINE.

## FLOTATION AGENT.

No Drawing.

Application filed June 7, 1924. Serial No. 718,674.

This invention relates to a flotation agent, which may be used for effecting concentration of metalliferous ores.

Several well known methods are in general use for concentrating ores, e. g., for increasing the percentage of metal-bearing mineral in the ore by the elimination of a portion of the gangue. In the widely used froth-flotation method the ore is first pulverized and then thoroughly mixed with a large volume of water to form a pulp. This pulp is run through a "flotation machine" in which by some convenient means there is produced a froth compound of gas or air bubbles and particles of the ore. A small quantity of a flotation agent, usually an oil, is introduced into the "flotation machine" while the pulp is being formed to produce a sufficiently voluminous and stable froth, and to enhance the selective action of the gas. The flotation oil, if properly chosen, coats or "wets" the particles of metallic lustre in preference to the particles of gangue. This oily film promotes the adherence of the particles to the surface of the gas bubble, and thus results in the selective action whereby the bubbles collect or concentrate the mineral-bearing particles on their surface. The froth formed by these bubbles can be readily separated from the large volume of water in which the gangue remains suspended, and this froth on proper treatment such as settling, etc., yields the concentrate.

A wide variety of flotation agents have been used since it has been found that different ores require various kinds and quantities of such agents. The most widely used flotation agents for copper ores are coal tars, coal-tar creosotes, cresylic acid and kerosene acid sludges,—other oils such as pine oil, etc., being frequently used in small quantities to increase frothing. Sulfuric acid is also used in large quantities as a supplementary agent to obtain a condition of acidity, which is frequently desirable. For lead and lead-silver ores hardwood creosote is employed in greatest quantity, followed by coal tars, crude petroleum and pine oils.

Two distinct properties are required of a flotation oil to obtain the desired results. First, the oil must stabilize the froth formed from the water, the gas and the solids of the pulp; second, it must selectively "wet" the metallic particles present in the pulp solids. To possess good frothing properties the oil

must be soluble in water and must diminish its surface tension. To possess selective properties the oil must be more readily absorbed on the surface of the metallic particles than on that of the gangue particles. 60 No oils will perform both of these functions equally satisfactorily with all ores and in all processes, and hence no flotation agent can be regarded as universally applicable.

The primary object of the present invention is to provide a flotation agent which is comparatively inexpensive, and by means of which a high grade concentration of many metal-bearing minerals can be satisfactorily recovered. 65

Another object of the invention is to provide a flotation agent the component parts of which can be readily varied to make it more effective for treating particular ores by different methods. 70

With these and other objects in view, the invention consists in the new flotation agents hereinafter described and particularly defined in the claims.

The flotation agent or composition forming the subject-matter of the present invention may be described as an oil containing one or more of three typical groups of compounds which are respectively acidic, basic, and neutral in their properties. The acidic group is composed of alkali-soluble organic hydroxy compounds or tar-acids, of which at least fifty percent boil above 220° C. These acidic compounds are analogous to the higher homologues of phenol which occur in very small quantities in ordinary coke-oven tar, but differ from them by having a larger content of hydrogen or more alkyl side chains, which give them a higher molecular weight, a lower refractive index, and a lower density for the same boiling point. The basic group is composed of hetero-cyclic unsaturated nitrogen bases, soluble in dilute acid. These basic compounds are analogous to the pyridine-quinoline-acridine series of ordinary coke-oven tar, but differ from them by having a larger content of hydrogen or more alkyl side chains, which give them a higher molecular weight, a lower refractive index, and a lower density for the same boiling point. 85

The neutral group is composed chiefly of cyclic unsaturated hydrocarbons, insoluble in alkali and dilute acid. They are genetically related to the benzene-naphthalene series of compounds of coke-oven tar, 100 105 110

but differ from them by having a larger content of hydrogen or more alkyl side chains, which give them a higher molecular weight, lower refractive index, and a lower density 5 for the same boiling point. The difference between these cyclic unsaturated hydrocarbons and the aromatic hydrocarbons present in ordinary coke-oven tar is shown by the fact that the unsaturated compounds decolorize dilute solutions of potassium permanaganate or bromine; whereas benzene, naphthalene and their homologues do not. 10

In its most widely applicable form the oil forming the subject-matter of this invention 15 consists of a mixture containing fifteen to forty-five per cent of the above described acidic compounds; one to six per cent of the above described basic compounds, and the balance of the above described neutral 20 compounds. However, the invention is not limited to these specific mixtures in these proportions, or containing all three of these component groups.

The several groups of compounds, a mixture of which in proper proportions comprises the invention, can be prepared from the primary or only partially decomposed primary tar obtained by distilling coal or other bituminous material under mild conditions of carbonization; such, for example, as those described in the United States patent to Henry L. Doherty, No. 1,426,159, granted August 15, 1922, or in the co-pending application of Henry O. Loebell, Serial 35 No. 640,828, filed May 23, 1923, entitled "Manufacture of water gas", but which conditions are quite different from those which give rise to coke-oven tar, the origin of many ordinary flotation oils. In either of 40 the processes described in the above application or patent, coal or other bituminous material is passed in a descending column through a shaft furnace and during its passage through one part of the furnace is progressively carbonized by a rising current of hot gases. The coal is gradually heated to higher temperatures, and its volatile constituents are carried away by the heating 45 gases without being exposed to temperatures much in excess of those required for their liberation. As a result of these mild conditions of carbonization the tar condensed from this gas consists of the primary or only partially decomposed liquid distillate 50 of the coal and is clearly distinguishable both in its physical and chemical properties 55 from ordinary coke-oven tar.

This primary tar has a lower density and 60 lower "free carbon" content and is radically different from coke-oven tar in its chemical composition. The primary tar and its various distillates commonly contain ten to fifty percent of relatively high boiling tar-acids; fifty to ninety percent of non-aromatic hydrocarbons, more than one-half of

which are unsaturated; and one to three percent of nitrogen bases. These tar-acids are not simply the well known higher homologues of phenol which occur in small quantities in ordinary coke-oven tar, but can be 70 regarded as hydrogenated and alkylated derivatives of these compounds. Moreover, whereas the hydrocarbons of coke-oven tar belong to the aromatic group and its nitrogen bases to the pyridine-quinoline-acridine 75 group, such compounds are not present in other than small amounts in primary tar or its distillates, but the primary tars contain their unsaturated derivatives with additional hydrogen and alkyl groups attached 80 to their nuclei.

The primary tar-acids can be isolated by extraction of the tar or its distillates with dilute caustic soda and acidification of the alkaline solution thus formed. The nitrogen bases can be isolated from the oil remaining after this tar-acid extraction by treating it with dilute mineral acid, a solution thus being obtained from which they 90 can be liberated. The residual neutral oil 95 remaining after extraction of the tar-acids and the nitrogen bases constitutes the hydrocarbons of this primary tar. These compounds are characterized by the presence in excess (one-half to four-fifths of the total) 95 of cyclic unsaturated hydrocarbons which are genetically related to the benzene-naphthalene series of compounds but have a larger content of hydrogen or more alkyl 100 groups.

The neutral oil which is thus obtained from primary or only partially decomposed primary tar, and which contains such cyclic unsaturated non-aromatic hydrocarbons, has proved in the case of many ores to possess 105 the properties of selecting the mineral-bearing metal, i. e., of coating it with an oily film in preference to so coating the gangue. The basic oil containing the nitrogen bases also possesses this selective action to a high 110 degree, but differs from the neutral oil in the ores with which it is most effective. It is believed that the superiority of these basic and neutral oils as selective agents can be 115 explained by the presence of "unsaturated" linkages in their molecules, by means of which there is promoted a differential adsorption at the surfaces of the mineral and gangue. Under certain conditions the cyclic 120 unsaturated hydrocarbon oils have a sufficient froth-forming capacity, but the more soluble basic compounds have been found to possess this property to a much greater extent. Hence these neutral and basic oils can 125 be used separately for flotation of certain kinds of ores, but when used together they usually give more satisfactory results.

In cases where the cyclic unsaturated oils and/or the nitrogen bases do not produce a satisfactory froth it has been found that 130

the addition to these oils of varying amounts of the high-boiling phenol-like compounds or tar-acids which are present in the primary tar oils greatly increases the frothing properties of the resultant oil. When a flotation oil comprising a mixture of cyclic unsaturated hydrocarbons and/or hetero-cyclic unsaturated nitrogen bases together with such high boiling phenol-like compounds is added to a pulp of pulverized ore and water, the tar-acids are distributed between the water and the oil. The comparatively insoluble neutral oil acts as a reservoir for the more soluble tar-acids and nitrogen bases, and reduces the diminution of their frothing power by dilution. Thus it has been found that by properly blending a mixture of cyclic unsaturated hydrocarbons, hetero-cyclic nitrogen bases, and phenol-like compounds, all of which possess some frothing power but which differ in their selectivity, i. e., "oiling" or "collecting" power, flotation oils can be prepared by means of which a wide variety of ores can be effectively concentrated.

It has also been found that the particular mixture of high-boiling phenol-like compounds which is present in primary tar oils of the class described is a considerably more effective frothing agent than the mixture of low-boiling and slightly more soluble phenols found in ordinary coke-oven tar. Moreover, this mixture also possesses selective properties to a degree such as to make its use alone feasible in concentrating many ores, without the addition of neutral oils or other agents excessively selective in their action. It is possible to add to this wide range of tar-acids occurring naturally in tar a fraction of the lower-boiling members of the series which are more soluble in water, and thus to modify the selective and frothing properties of the resultant oil.

The differences in constitution between a coke-oven tar and a primary tar such as is produced by the Doherty or Loebell processes have been discussed, and it is these differences which are believed to be responsible for the pronounced improvements thus made in the technology of ore concentration. A cheaper flotation agent is made possible because these primary tars contain naturally a far higher percentage of the desirable phenol-like compounds than do coke-oven tars. Moreover, it has been found that the selective properties and frothing ability of oil from this source are superior to those of flotation agents available at present. The distillates of such primary tar contain these tar acids, bases, and neutral oils naturally in about the proportions which are effective in promoting flotation under the conditions most often encountered. Moreover, almost any other combination can be prepared at little expense from these acidic, basic and

neutral components to meet special conditions, and since all of the various mixtures prepared from these primary tar oils have a much lower viscosity than the corresponding fractions from coke-oven tar they can be more readily and completely disseminated through the pulp and hence are far more efficient flotation agents.

Although the invention has been described with reference to the high boiling tar-acids or phenol-like compounds and the cyclic unsaturated hydrocarbons and hetero-cyclic nitrogen bases which are recovered from a primary or only partially decomposed primary tar such as that produced by the Doherty or Loebell processes, it is not intended to limit the invention to the use of specific tar produced in these two processes or to its distillates or acidic, basic, and neutral oil components. It is apparent that any hydrogenated and alkylated derivatives of the higher homologues of phenol of which at least fifty per cent boil above 220° C.; that any hetero-cyclic unsaturated nitrogen bases which are hydrogenated and alkylated derivatives of the pyridine-quinoline-acridine series; and that any cyclic unsaturated hydrocarbons which are the similar derivatives of the benzene-naphthalene-anthracene series, can be used and combined in making flotation agents having similar properties.

The term "phenol-like compounds" has been chosen to define the mixture of tar-acids or alkali-soluble organic hydroxy-compounds which are present in the above described primary or only partially decomposed primary tar. It is to be understood, therefore, that the term "phenol-like compounds" is used in the claims as a generic term to cover compounds analogous to or prototypes of ordinary phenols, such as the hydrogenated or alkylated derivatives of the homologues of phenol, naphthol and polycyclic phenolic compounds.

The preferred form of the invention having been thus described, what is claimed as new is:

1. A flotation agent containing cyclic unsaturated hydrocarbons which are the hydrogenated and alkylated derivatives of aromatic hydrocarbons.
2. A flotation agent containing a mixture of cyclic unsaturated derivatives of aromatic hydrocarbons together with phenol-like compounds of which at least fifty per cent by volume boil above 220° C.
3. A flotation agent containing a mixture of cyclic unsaturated derivatives of aromatic hydrocarbons and their homologues together with hetero-cyclic unsaturated nitrogen bases.
4. A flotation agent containing hetero-cyclic unsaturated nitrogen bases together with phenol-like compounds of which at

least fifty per cent by volume boil above 220° C.

5. A flotation agent containing high boiling phenol-like compounds, hetero-cyclic unsaturated nitrogen bases and cyclic unsaturated derivatives of the aromatic hydrocarbons.

6. A flotation agent containing fifteen to

forty-five per cent by volume of high boiling phenol-like compounds, one to six per 10 cent by volume of hetero-cyclic unsaturated nitrogen bases, and more than twenty-five per cent by volume of cyclic unsaturated hydrocarbons.

In testimony whereof I affix my signature.

ALBERT L. KLEES.